

Oct. 20, 1942.

J. R. GIER, JR

2,299,138

HEAT TREATING OF STEEL

Filed Oct. 4, 1941

2 Sheets-Sheet 1



WITNESSES:

Paul C. Groome

INVENTOR

John R. Gier, Jr.

BY

James M. Ely

ATTORNEY

Oct. 20, 1942.

J. R. GIER, JR

2,299,138

HEAT TREATING OF STEEL

Filed Oct. 4, 1941

2 Sheets-Sheet 2



INVENTOR  
John R. Gier, Jr.  
By James M. Ely  
ATTORNEY

## UNITED STATES PATENT OFFICE

2,299,138

## HEAT TREATING OF STEEL

John R. Gier, Jr., Wilkinsburg, Pa., assignor to  
Westinghouse Electric & Manufacturing Com-  
pany, East Pittsburgh, Pa., a corporation of  
Pennsylvania

Application October 4, 1941, Serial No. 413,625

6 Claims. (Cl. 148—17)

This invention relates to the heat treating of steel, and particularly to a method of hardening stainless steel.

This application is a continuation-in-part of my copending applications Serial Nos. 296,586 and 296,587, which were filed September 26, 1939, entitled Heat treating furnaces, now issued as Patents Nos. 2,290,551 and 2,290,552, respectively, and which are assigned to the same assignee as this invention.

Many types of mechanical devices operate in such a way that failure, corrosion or wear on one or more surfaces may cause serious functional breakdown of the mechanism. Particularly in outdoor or marine applications, it is necessary to provide certain mechanical devices which are maintained free from rust, have sufficient hardness to resist wear, have sufficient impact strength to resist chipping or breaking, and have a uniformity of frictional coefficient.

Heretofore, different methods of heat treating metals have been employed to give them improved characteristics. Nitriding of steel has greatly extended the range of service life on many wearing parts because of the combination of unusually high hardness and wear resistance characteristics which are obtainable while at the same time obtaining moderate corrosion resistance and low frictional characteristics. However, where the nitrided steels are employed where concentrated loads or impact stresses are encountered, particularly at edges and sharp corners, chipping and spalling of the nitrided case are encountered. Other known processes, such as case carburization, have not been employed to give toughness to the steel except where corrosion resistance is not a factor.

In marine or seaboard service, it is often necessary to employ stainless steel in many of the applications because of its corrosion resistance. This corrosion resistance of the stainless steel is provided throughout the cross-section of the part formed therefrom but is accompanied by a decrease in wear resistance. The stainless steel parts invariably have low uniform frictional characteristics rendering them especially suitable for applications such as engaged latches which must be disengaged by a calibrated slowly applied load. However, because of the lack of toughness and low wear resistance, the use of stainless steel in such applications has not found universal favor.

It is an object of this invention to provide for increasing the wear resistance of stainless steel.

Another object of the invention is to simul-

taneously effect the case carburization and the bright hardening of stainless steel.

Other objects of this invention will become apparent from the following description when taken in conjunction with the accompanying drawings, in which:

Figures 1, 2, 3, 4, 5 and 6 are graphs, the curves of which illustrate the effect of variations in the composition of the gaseous atmosphere on the hardness gradient of the steel treated in accordance with this invention;

Figs. 7, 8 and 9 are graphs, the curves of which illustrate the effect of time and temperature of treatment on the hardness gradient of another steel treated in accordance with this invention;

Figs. 10, 11 and 12 are graphs, the curves of which illustrate the effect of time and temperature of treatment on the hardness gradient of a different steel treated in accordance with this invention; and

Fig. 13 is a graph, the curves of which illustrate the effect of variations in the gaseous atmosphere on the hardness gradient of the stainless steel treated in accordance with this invention.

In practicing this invention, excellent results are obtained where a protective atmosphere, formed of extremely pure dissociated ammonia to which from 0.4% to 2% of methane is added, is employed. Good results have also been obtained where up to 3% of methane is added to the dissociated ammonia in forming the protective atmosphere.

The method of this invention is particularly applicable to stainless steel articles having a chromium content of 10 to 15% and a carbon content of 0.5 to .90%. It is especially applicable to stainless steel articles having a preferred composition of 11.5% to 14% chromium, .10% to .36% carbon, less than .5% of each of manganese, silicon and phosphorus, with the balance iron, except for incidental impurities.

In practicing this invention, the steel articles having the composition given hereinbefore are subjected to a heat treatment which normally effects the bright hardening thereof. This treatment consists preferably of heating the stainless steel articles in a protective atmosphere at a temperature between 825° C. and 1040° C. for a predetermined period of time of between 15 minutes and three hours, and effecting an atmospheric quenching or cooling of the articles in the protective atmosphere from the heating temperature.

The methane added may be pure methane or may be added in the form of natural gas which, as is well known, contains about 85% of methane.

The methane is preferably mixed with the pure dissociated ammonia prior to being admitted to the heating chamber in which the stainless steel articles are treated.

The heat treatment of the stainless steel articles is preferably done in a furnace of the type disclosed and claimed in my Patent No. 2,290,552 which issued July 21, 1942, entitled Heat treating furnaces, and in which provision is made for withdrawing the articles from the heating chamber to a quenching or cooling chamber in which the articles are caused to be quickly cooled while enveloped in an atmosphere of the same composition as the protective atmosphere within the heating chamber. Other furnaces, and particularly furnaces of the type disclosed in the copending application of W. E. Mahin, Serial No. 416,181, filed October 23, 1941, may, however, be utilized as long as provision is made for obtaining and admitting the mixture of pure dry dissociated ammonia and methane, the mixture having a low dew point of  $-60^{\circ}$  C. to  $-80^{\circ}$  C., into the heating chamber and the quenching chamber and preventing contamination of the protective atmosphere within the furnace. In practicing this invention, it is important to maintain the low dew point of  $-60$  to  $-80^{\circ}$  C. for the purpose of bright finishing the steel and for maintaining the carburizing power of the protective atmosphere.

When the stainless steel articles are treated in the protective atmosphere as described, it is found that a simultaneous bright finishing and case carburization of the articles is effected. The treated stainless steel has an extremely bright surface, a definite case hardness and a very tough core.

The hardness of the case and the depth of the case are affected by the amount of methane mixed with the dissociated ammonia, the temperature at which the steel is treated and the length of time of such treatment, as is clearly illustrated by the curves of Figs. 1 through 13 of the accompanying drawings.

Referring to Fig. 13, there is illustrated the hardness gradient curves obtained on a .30% carbon type of stainless steel having the specific analyses of .36% carbon, 13.96% chromium, 0.34% manganese, 0.12% silicon, 0.02% phosphorus and the balance iron and incidental impurities when subjected to the heat treatment consisting of heating the steel at a temperature of  $1010^{\circ}$  C. for one hour in the protective atmosphere, then quickly cooling the steel while enveloped and protected by the protective atmosphere. Curve 10 illustrates the hardness gradient obtained where .05% of natural gas, equivalent to 0.42% methane, is added to the dissociated ammonia to form the protective atmosphere while curve 12 illustrates the hardness gradient obtained with a steel of the same analyses and treated in the same manner, except that 3.0% of natural gas, equivalent to 2.55% methane, is added to the dissociated ammonia to form the protective atmosphere. As illustrated, the increase in the methane content of the protective atmosphere increases the case hardness imparted to the stainless steel without detracting from the toughness of the core.

Referring to Figs. 1, 2, 3, 4, 5 and 6, there is illustrated the effect of additions of methane to the protective atmosphere on the case hardness of a 0.10% carbon type stainless steel having the specific analyses of 0.12% carbon, 13.32% chromium, 0.30% manganese, 0.56% silicon, 0.01% phosphorus, and the balance iron and incidental

impurities. In these figures, curves 14, 16, 18, 20, 22 and 24 of Figs. 1, 2, 3, 4, 5 and 6, respectively, illustrates the effect of variations of the methane content of the protective atmosphere on the hardness gradient. The hardness gradient illustrated by curves 14, 16, 18, 20, 22 and 24 is obtained where 0.5%, 1%, 1.5%, 2%, 2.5% and 3%, respectively, of natural gas is added to the dissociated ammonia with the heat treating cycle comprising heating the steel at a temperature of  $1010^{\circ}$  C. for a period of one hour, after which the steel is cooled while enveloped in the respective protective atmospheres. Curves 26, 28, 30, 32, 34 and 36 of Figs. 1 through 6, respectively, illustrate the hardness gradient obtained where the steel is heated at a temperature of  $1010^{\circ}$  C. for a period of one hour in the dissociated ammonia protective atmosphere containing natural gas additions in the amount of 0.5%, 1%, 1.5%, 2%, 2.5% and 3%, respectively, and cooled in the furnace atmosphere, after which the steel is cooled in dry ice at a temperature of  $-78^{\circ}$  C.

Upon examining the 0.10% carbon type of stainless steels treated in the manner described and in which the protective atmosphere contains different amounts of methane, it is found that appreciable carbon concentration at the surface of the steel caused austenite retention, the degree depending upon the amount of carburization which occurs. For this reason, the specimens were tested for hardness both before and after cooling in dry ice to effect at least a partial transformation of the austenite. An examination of the results illustrated in Figs. 1 through 6 reveals that where this particular steel is treated in a protective atmosphere containing more than 1% methane, excessive amounts of retained austenite are obtained resulting in low hardness at or near the surface of the stainless steel article.

Referring to Figs. 7, 8 and 9, there is illustrated the effect of the heat treatment of this invention on the hardness gradient curves for a 0.30% carbon type stainless steel having the specific analyses of 0.36% carbon, 13.96% chromium, 0.34% manganese, 0.12% silicon, 0.02% phosphorus, and the balance iron and incidental impurities. These curves primarily show the effect of time and temperature of treatment on the hardness gradient, the curves of Fig. 7 illustrating the hardness gradient when the steel is subjected to the heat treatment at different temperatures for  $\frac{1}{2}$  hour, the curves of Fig. 8 illustrating the effect of the treatment at different temperatures for a period of time of 1 hour, and the curves of Fig. 9 illustrating the effect of the treatment at different temperatures for a period of time of  $2\frac{1}{2}$  hours. In all cases, the heat treatment was effected in a protective atmosphere consisting of pure dissociated ammonia containing 1% of natural gas, which is equivalent to .85% of methane.

In the drawings, curves 37, 38 and 39 of Figs. 7, 8 and 9, respectively, illustrate the hardness gradient for this particular steel when the heat treatment includes heating the steel at a temperature of  $900^{\circ}$  C. Curves 40, 41 and 42 of Figs. 7, 8 and 9, respectively, illustrate the hardness gradient obtained where the heating temperature is  $950^{\circ}$  C. Curves 43, 44 and 45 of Figs. 7, 8 and 9, respectively, illustrate the hardness gradient on the same steel when the heat treatment includes heating at a temperature of  $1000^{\circ}$  C., while curves 46, 47 and 48 of Figs. 7, 8 and 9, respectively, represent the hardness gradient of the steel when the steel is subjected to a treat-

ment including heating at a temperature of 1040° C. From the curves of Figs. 7, 8 and 9, it is evident that for a given temperature, the maximum hardness increases with time at the lower temperatures but at the higher temperatures austenite retention results in the development of low surface hardness.

Referring to Figs. 10, 11 and 12, there is illustrated the effect of time and temperature of the heat treatment of this invention on the hardness gradient curves for a 0.10% carbon type of stainless steel having the specific analyses of 0.12% carbon, 13.32% chromium, 0.30% manganese, 0.56% silicon, 0.01% phosphorus and the balance iron and incidental impurities. The curves of Fig. 10 are based on steel which has been subjected to a treatment in dissociated ammonia containing .85% methane for a period of time of  $\frac{1}{2}$  hour at a heating temperature, whereas the curves of Figs. 11 and 12 were obtained for treatments in the same protective atmosphere at heating temperatures for a period of time of 1 hour and  $2\frac{1}{2}$  hours, respectively.

In the drawings, curves 49, 50 and 51 of Figs. 10, 11 and 12, respectively, are representative of the hardness gradient obtained where the heat treatment included heating at a temperature of 900° C., while curves 52, 53 and 54 of Figs. 10, 11 and 12, respectively, represent the hardness gradient obtained where the heat treatment included heating at 950° C. Curves 55, 56 and 57 of Figs. 10, 11 and 12, respectively, illustrate the hardness gradient for the different periods of time of heat treatment at a temperature of 1000° C., while curves 58, 59 and 60 of Figs. 10, 11 and 12, respectively, are representative of the results obtained where the heating temperature was 1040° C. The curves of Figs. 10, 11 and 12 illustrate the same tendencies as the tests in which the amount of methane in the atmosphere is varied, that is, when the carbon at the surface reached a concentration resulting in a hardness of approximately 700 Vickers austenite retention begins to occur, and further carburization causes lower hardness. This is particularly true at the higher temperatures which promote austenite retention.

The heat treatment of this invention improves the transverse breaking strength of the stainless steel articles. For example, a stainless steel having a carbon content of 0.37% and a chromium content of 12.6% by analyses has a breaking strength of 189,000 lbs. per square inch after having been treated for one hour at a temperature of 1010° C. in pure dissociated ammonia. When the same steel is heated for the same period of time, and at the same temperature in the protective atmosphere utilized in the method of this invention consisting of dissociated ammonia and 1% of methane, the breaking strength is increased to 260,000 lbs. per square inch. At the same time, the Rockwell "C" hardness of the steel after being subjected to the respective treatments, is 58 and 62, respectively, the higher hardness being obtained through the use of the protective atmosphere containing methane.

As another example of improvement in the hardness of steel when treated in accordance with this invention, the surface hardness of the low carbon (0.12%) martensitic stainless steels is increased to as high as 66 Rockwell "C" with no apparent decrease in corrosion resistance when heat treated in the protective atmosphere of dissociated ammonia and from 1 to 2% of free methane thereby providing a high surface hardness and a tough, impact resisting core.

The method of this invention is effective for simultaneously producing a bright finish and case carburization of the stainless steels. This method finds particular application in the bright hardening of stainless steel articles such as springs, triggers, latches, levers, pins, small gears, or the like, which are subjected to impact stresses, and at the same time provides articles having corrosion resistance, excellent wear resistance, freedom from spalling and marked uniformity of frictional coefficient.

I claim as my invention:

1. In the method of case hardening stainless steel containing from .05% to .90% carbon and 10% to 15% chromium, in combination, the step of heating the steel in an atmosphere comprising dissociated ammonia and from 0.4% to 3% of methane.
2. In the method of case hardening stainless steel containing from .05% to .90% carbon and 10% to 15% chromium, in combination, the step of heating the steel in an atmosphere comprising dissociated ammonia and about 1% of methane.
3. The method of claim 1 in which the steel is heated for a period of time of from 15 minutes to 3 hours at a temperature between 825° C. and 1040° C.
4. In the method of case hardening stainless steel containing from .05% to .90% carbon and 10% to 15% chromium, in combination, the steps of, heating the steel in an atmosphere comprising dissociated ammonia and from 0.4% to 3% of methane at a temperature between 825° C. and 1040° C., and cooling the steel in the atmosphere containing methane.
5. The method of case hardening stainless steel containing from .05% to .90% carbon and 10% to 15% chromium comprising, heating the steel in an atmosphere comprising dissociated ammonia and from 0.4% to 3% of methane for a period of time of from 15 minutes to 3 hours at a temperature between 825° C. and 1040° C., and cooling the steel in the atmosphere of dissociated ammonia and methane to provide a hard outer case on the steel free from tarnish or scale.
6. In the method of heat treating stainless steel containing from .05% to .90% carbon and 10% to 15% chromium, in combination, heating the steel in a gaseous atmosphere comprising dissociated ammonia and from 0.4% to 3.0% methane at a temperature between 825° C. and 1040° C., the gaseous atmosphere having a dew point between  $-60^{\circ}$  C. and  $-80^{\circ}$  C., and cooling the steel in the gaseous atmosphere.